

D. R. McARTHUR,

METHOD OF MAKING A HYDROCARBON LIQUID SUITABLE FOR USE IN INTERNAL  
COMBUSTION ENGINES.

APPLICATION FILED JUNE 28, 1913.

1,119,974.

Patented Dec. 8, 1914.



Attest.  
Mehring Stahl  
C. E. Parsons

*Inventor.*  
Donald R. McArthur

By Sean Middleton Donaldson Jr.  
S.M.D.

# UNITED STATES PATENT OFFICE.

DONALD R. McARTHUR, OF BRADFORD, PENNSYLVANIA, ASSIGNOR OF TWO-THIRDS  
TO EDGAR W. TAIT, OF BRADFORD, PENNSYLVANIA.

## METHOD OF MAKING A HYDROCARBON LIQUID SUITABLE FOR USE IN INTERNAL- COMBUSTION ENGINES.

1,119,974.

Specification of Letters Patent.

Patented Dec. 8, 1914.

Application filed June 28, 1913. Serial No. 776,299.

*To all whom it may concern:*

Be it known that I, DONALD R. McARTHUR, a citizen of the United States, residing at Bradford, Pennsylvania, have invented certain new and useful Improvements in the Method of Making a Hydrocarbon Liquid Suitable for Use in Internal-Combustion Engines, of which the following is a specification.

10 My invention consists of certain new and useful improvements in the art or method of making a hydrocarbon liquid suitable for use in internal combustion engines.

15 My process consists in exposing to compression and the heat resulting from compression natural gas and commingling it with a higher liquid paraffin, and then cooling and collecting the resultant to form a liquid of lower specific gravity than that of 20 the higher liquid paraffin.

25 In carrying out my process I compress, by any known method of compression, natural gas to a pressure of one hundred pounds per square inch or more, (the exact pressure 30 preferable depending on the quality of the natural gas used and on the desired specific gravity of the product). At a point a few inches from where the compressed gas leaves the compressor, or at any further point 35 where the necessary heat is still maintained I commingle with the natural gas kerosene, naphtha or other higher paraffins in either a liquid or gaseous form, preferably by injecting the higher paraffin by means of a 40 force pump or other device. I inject this higher paraffin preferably through a smaller tube of about half the diameter of the pipe carrying the compressed natural gas; the length of this tube varies according to the 45 quality of the natural gas used and according to the rapidity with which the compressed gas is traveling through the system; at the end of this tube is a hole or "needle valve" through which the higher paraffin 50 escapes into, and commingles with, the compressed natural gas; it is preferable, and better results may be obtained, if the needle-valve is so adjusted that it will not allow the higher paraffin to escape through it until there is a considerably greater pressure 55 in the tube through which the higher paraffin is passing than there is in the pipe through which the compressed natural gas is passing, the effect being to keep the

higher paraffin before it is commingled with the natural gas at a constant pressure greater than the pressure on the natural gas; good results have been obtained by maintaining in the tube a pressure one hundred pounds higher than in the larger pipe through which the compressed natural gas is traveling. I then cool and collect the commingled hydrocarbons, the hydrocarbons of the natural gas being condensed into a liquid with the hydrocarbons of the higher paraffin used, and the resultant being a hydrocarbon liquid suitable for use in internal combustion engines. The cooling and collecting may be effected by any known method, such as passing the commingled hydrocarbons through a long worm of pipe until they are sufficiently cooled, thence into a receiving tank; additional cooling may be had by expanding the compressed unconsumed gas in the tank into a tank or pipe incasing the worm in which the commingled hydrocarbons are traveling.

The accompanying drawing represents a diagrammatic view of means for carrying out my process.

In this drawing the gas inlet is shown at A entering a tank B where its impurities are deposited; thence the natural gas passes through pipe C to a compressor D and thence through a pipe E.

85 The oil tank is shown at F and the oil pump at G, an engine H operating both the compressor and the pump preferably. The oil is conveyed through a pipe I and through the tube N which is inserted within the pipe K. At the end of tube N is a valve O which retains a pressure of several pounds more on the oil in the tube N than on the gas in pipe K, before it releases the oil into pipe K where it commingles with the compressed natural gas which has been traveling in pipe K. While in the tube N the oil is heated by the hot gas surrounding the tube N, and after the oil and gas are commingled the commingled substances are further subjected to the heat resulting from the compression of the natural gas. From the point of commingling the commingled substances are conveyed through a pipe K to cooling pipes L, and thence the hydrocarbon liquid suitable for use in internal combustion engines passes into tank M.

100 In carrying out my process I secure ad-

ditional cooling by jacketing part of the condenser as shown at *a*, and this jacket is connected at one end with the tank *M* through a pipe *b* and a relief valve *c*, and at the other end to an exhaust pipe *d*, so that what gas may flow into tank *M* will pass out through pipe *b* and the space between the jacket and its inclosed section of the condenser and through the exhaust, and this gas may be discharged into the atmosphere or utilized as fuel in the engine.

A typical instance of operating my process would be as follows: I introduce natural gas into the compressor at the rate of 4,000 cubic feet per hour. In the first or low stage of the compressor the gas is compressed to a pressure of about 40 pounds per square inch; it passes thence into the second or high stage of the compressor where additional compression is had. The oil or other paraffin is injected into the compressed natural gas at the rate of about 40 gallons per hour. This oil may be a naphtha of 50° to 56° Baumé gravity, or it may be a heavier oil. The relief valve is set so that a pressure of 225 pounds per square inch is maintained on the system. The valve at the end of the tube *N* is set so that there is a pressure of 350 pounds per square inch on the oil in the tube *N*. The cooling system is composed of pipe two inches in diameter and about 800 feet in length, of which the last 200 feet are incased or jacketed. The relief valve *c* releases the unconsumed gas in the receiving tank whenever the pressure on the receiving tank reaches 225 pounds per square inch. Better results are obtained when using natural gas containing a high percentage of ethane or higher paraffins.

40 What I claim and desire to secure by Letters Patent is:

1. The process of making a hydrocarbon liquid suitable for use in internal combustion engines by subjecting to compression and exposing to the heat resulting from the compression, compressed natural gas and commingling it with a higher liquid par-

affin, and then cooling and collecting the resultant to form a liquid of lower specific gravity than that of the higher liquid 50 paraffin.

2. The process of making a hydrocarbon liquid suitable for use in internal combustion engines by subjecting to compression and exposing to the heat resulting from the compression, compressed natural gas and commingling it with an atomized or vaporized higher paraffin, and then cooling and condensing the resultant to form a liquid of lower specific gravity than that of the 60 higher paraffin.

3. The process of making a hydrocarbon liquid suitable for use in internal combustion engines by compressing natural gas and subjecting to a greater pressure a higher 65 liquid paraffin, and subjecting the higher liquid paraffin while under the greater pressure to the heat resulting from the compression, and then, while the proper degree of heat is still maintained, mingling in proper 70 proportion the compressed natural gas and the higher liquid paraffin, and then cooling and collecting the resultant to form a liquid of lower specific gravity than that of the 75 higher liquid paraffin.

4. The process of making a hydrocarbon liquid suitable for use in internal combustion engines by compressing natural gas and subjecting to a greater pressure an atomized or vaporized higher paraffin, and, while the proper degree of heat is still maintained on the natural gas and the higher paraffin, mingling in proper proportion the compressed natural gas and the higher paraffin, and then cooling and condensing the 85 resultant to form a liquid of lower specific gravity than that of the higher paraffin.

In testimony whereof, I affix my signature in presence of two witnesses.

DONALD R. McARTHUR.

Witnesses:

KATHARINE BURKE,  
EDGAR W. TAIT.